

## UNITED STATES PATENT OFFICE

2,200,452

## METHOD OF PRODUCING CELLULOSIC FIBERS HAVING AFFINITY FOR ACID DYES

Karl Kösslinger, Dessau, Hermann Klare, Wolfen  
Kreis Bitterfeld, and Herbert Rein, Dessau,  
Germany, assignors to I. G. Farbenindustrie  
Aktiengesellschaft, Frankfort - on - the - Main,  
Germany

No Drawing. Application May 9, 1935, Serial  
No. 20,704. In Germany May 15, 1934

2 Claims. (Cl. 8—116)

One of its objects is an improved process of this kind. Another object is to improve the capacity of vegetable or artificial cellulosic fibers to be dyed by acid dyes as used for dyeing wool. 5  
5 Further objects will be seen from the detailed specification following hereafter.

According to this invention a good affinity for said wool-dyestuffs is imparted to vegetable or artificial cellulosic fibers by incorporating in the 10 fiber, according to the customary methods, a primary, secondary or tertiary amine of the general formula  $(R_1, R_2, R_3)N$  or a quarternary ammonium base of the general formula:  $(R_1, R_2, R_3, R_4)N\text{OH}$  or a salt of any of these 15 compounds. These substances react on the fiber with the dyestuff acid and thus fix the dyestuff to the cellulosic fiber, so that they give to cotton, artificial silk and other cellulosic fibers dyeing properties similar to those of animal fibers. It 20 is essential for the purpose of the invention that the amine or ammonium base should be taken up and retained by the fiber; this is the case when at least one of the residues represented by  $R_1, R_2, R_3$  and  $R_4$  comprises an aliphatic chain having eight or more carbon atoms. The remaining 25 groups in the amine or ammonium base may be hydrogen, aromatic residues or aliphatic residues containing less than eight carbon atoms. The nitrogen atom of the amine or ammonium base 30 may itself be a member of a ring system, that is to say it may belong to a heterocyclic ring.

The compounds may be incorporated in the cellulosic fibers by impregnating the fiber with a solution or emulsion of the base or of a salt thereof or with an inorganic or organic acid. An addition 35 of formaldehyde increases the fastness of the dyeings produced on fibers treated in accordance with the invention. The formaldehyde may be added to the impregnating bath or it may be applied to the fibers in a separate bath.

Instead of introducing the compounds subsequently to the production of the artificial fibers, the amine or ammonium base or salt thereof may be incorporated in the spinning solution and the latter then spun according to the known methods. Since the compounds are contained in the 45 artificial fibers thus produced, the same effect is attained. The effect is further improved by the simultaneous addition of proteins to the spinning solution directly before the spinning in accordance with the process described in the U. S. Patent 2,059,632 to Paul Esselmann and Karl Kösslinger, one of these being also an in-

ventor of the present invention. These proteins may be fixed by the addition to the spinning solution of suitable compounds, for instance, cholic acid or acid amines such as formamide or acetamide. In this case also the amine or 5 ammonium base or salt thereof may be incorporated in the spinning solution or artificial fibers prepared according to the aforesaid patent may be subsequently treated with a solution or emulsion of the base or a salt thereof. 10

The following examples illustrate the invention:

*Example 1.*—200 grams of stearylamine acetate are dissolved in 40 liters of water containing 5 per cent of formaldehyde, 2 kilos of cellulosic artificial silk or cotton are introduced into the bath thus prepared and frequently moved therein upwards and downwards during 15 to 20 minutes. The material is then centrifuged and dried at 20 80 to 90° C. 20

*Example 2.*—The procedure is as in Example 1 with the exception that instead of stearylamine acetate there are used 20 grams of isopropyl-dodecylamine lactate or 200 grams of N-dodecyl-1:3-propylene diamine formate. 25

The term cellulosic is intended to include materials consisting of cellulose or cellulose hydrate, however, it shall exclude cellulose derivatives such as cellulose esters and ethers. 30

What we claim is:

1. A method of increasing the affinity of cellulosic fibers for acid dyes which method comprises treating the undyed fibers with formaldehyde and an aqueous liquid containing a compound selected from the group consisting of amines containing an aliphatic radical of more than 8 carbon atoms, tetra alkyl ammonium bases containing at least one radical with more than 8 carbon atoms and salts of these compounds, and drying the fibers thus treated. 35

2. A method of increasing the affinity of cellulosic fibers for acid dyes which method comprises impregnating the undyed fibers with formaldehyde and an aqueous liquid containing a compound selected from the group consisting of amines containing an aliphatic radical of more than 8 carbon atoms, tetra alkyl ammonium bases containing at least one radical with more than 8 carbon atoms and salts of these compounds, and drying the fibers thus treated. 40 45

KARL KÖSSLINGER.  
HERMANN KLADE.  
HERBERT REIN.